

Feb. 25, 1936.

P. R. JUDY

2,032,322

FLUX COATED ELECTRODE

Filed April 10, 1934

Fig. 1.



Fig. 2.

Inventor  
PAUL R. JUDY,  
Schenley & Trask  
Attn  
Attorneys

## UNITED STATES PATENT OFFICE

2,032,322

## FLUX-COATED ELECTRODE

Paul R. Judy, Muncie, Ind., assignor to Indiana  
Steel & Wire Company, Muncie, Ind., a corpo-  
ration of Indiana

Application April 10, 1934, Serial No. 719,846

2 Claims. (Cl. 219—8)

It is the object of my invention to produce a flux-coated electrode or weld-rod in which the flux-coating not only facilitates the welding operation and protects the welding during its making and forms only an easily removable slag, but also one in which such flux coating is made of readily obtainable and inexpensive materials.

In arc welding, as is well known, it is desirable to protect the molten metal both while it is being transferred from the electrode to the work and while the deposited metal is solidifying and cooling; and to provide in the coating the necessary ingredients to accomplish this purpose. To protect during the solidifying and cooling, it is desirable to provide on the molten metal a thin film of protective material, and to have this film substantially continuous and unbroken until the metal has solidified and cooled; but to have the film of such character that when the whole is cold such film is quite friable and easily removable. By maintaining the film unbroken while the weld-metal is liquid, unevenness of the surface and of the boundary of the weld is in large measure avoided. While the same materials which protect the deposited metal also serve to some extent to protect the metal as it is being deposited from the electrode, this latter protection may be more effectively obtained by providing a non-oxidizing gaseous envelope for the metal as it is being deposited; and this gaseous envelope can be obtained by providing in the weld-rod coating an organic material, such as wood flour, which burns to yield carboniferous gases, such as carbon dioxide.

I have discovered that I can obtain the desired results by providing in the weld-rod coating a mixture of ilmenite with an aluminum-bearing alkali-metal or alkaline-earth silicate, especially feldspar or mica; and binding the mixture together and to the weld-rod core by a silicate binder, such as sodium silicate. The aluminum-bearing silicate may also contain other metals in addition to alkali metals and alkaline earths, for instance iron. The ilmenite serves to maintain an unbroken protective film while the deposited metal is liquid and until it has solidified and cooled. Although either the ilmenite alone or (usually) the aluminum-bearing silicate alone is not friable, and tends in general to yield a slag which is hard to remove, even with sodium silicate present, the co-presence of the ilmenite and the aluminum-bearing alkali-metal or alkaline-earth silicate, such as feldspar or mica, makes a resultant slag which is quite friable and easily removable.

In addition to these three fundamental ingredients, I may and desirably do provide other ingredients in the coating. The chief among these is an organic material, such as wood flour. Others may be ferro-manganese and gum arabic; but they are relatively secondary.

The accompanying drawing shows a coated welding electrode or weld-rod embodying my invention: Fig. 1 is an elevation of such a coated welding electrode, partly broken away to show a longitudinal section; and Fig. 2 is a cross-section of such coated welding electrode, on the line 2—2 of Fig. 1.

In such drawing, the metallic wire or rod 10, usually a ferrous wire or rod of desired composition, is covered for all or the greater part of its length by a coating 11; and this coating is made of the mixture of ilmenite and an aluminum-bearing alkali-metal or alkaline-earth silicate, with a binder silicate (such as sodium silicate), desirably with wood flour, ferro-manganese, and gum arabic also present, as described above.

The ilmenite, which is an iron titanate is suitably reduced to a powder, for intimate mixing with the other ingredients used.

The aluminum-bearing silicate is also reduced to a powder, as by grinding, for intimate mixture with the other ingredients. It is most conveniently either feldspar or mica; but other aluminum-bearing alkali-metal or alkaline-earth silicates may be used, such as feldspathoids, zeolites, or epidotes. Various feldspars may be used, such as orthoclase, albite, oligoclase and labradorite; and various micas, such as biotite, muscovite, lepidolite, margarite, phlogopite, etc.

The binder silicate is desirably either sodium silicate or potassium silicate; desirably in the form of water glass if sodium silicate is used, or of the analogous substance if potassium silicate is used.

These three ingredients may vary widely in their relative proportions. The ilmenite and the aluminum-bearing silicate may each vary from 10% to 40% of the whole formed by these three ingredients, with the binder silicate (sodium silicate) forming the residue of that whole. An effective proportion is with the ilmenite and the feldspar or mica each forming 25% of that whole, and the sodium silicate (computed after it has lost its water) forming 50% of that whole.

Wood flour, or other powdered organic material, may be added in desirable amount; conveniently in the proportions of 15% to 50% of the total weight of ilmenite and the silicates.

Ferro-manganese, in powdered form, is also

desirably added in the coating. It has a multiple action. It supplies manganese which may be lost during the welding operation. It helps in forming the protecting coating. It also has a deoxidizing action, to protect against oxygen which may enter the heated space. It may vary in amount, but conveniently forms between 10% and 40% of the total weight of ilmenite and the silicates.

10 Gum arabic is also a desirable ingredient. It has several functions. Among these are that it helps in the binding action, and also helps in furnishing the carbonaceous gases. It usually is present in relatively small amount, such as 2% to 15% of the total weight of ilmenite and the silicates.

15 I give below an example of a coating mixture which I have found very effective, and which embodies all of the ingredients discussed above, although not all of them are necessary:

|                                                                                        | Percent  |
|----------------------------------------------------------------------------------------|----------|
| Ilmenite                                                                               | 10 to 40 |
| Aluminum-bearing alkali-metal or alkali-line-earth silicate (such as feldspar or mica) | 10 to 40 |
| Sodium silicate (dry basis)                                                            | 20 to 60 |
| Wood flour                                                                             | 10 to 30 |
| Ferro-manganese                                                                        | 5 to 15  |
| Gum arabic                                                                             | 1 to 5   |

In making the coating mixture, the ingredients are suitably mixed in the desired proportions, and applied to the electrode-core in any suitable manner, as by being extruded thereon. The rod which has thus been coated is suitably dried, and is used in the usual manner of welding electrodes. It can be effectively used in all positions, not only in the so-called down-hand welding, in which the work is below the electrode, but also for welding on vertical surfaces and in overhead welding. Also, the electrode is found not only to work with "reverse polarity", or when it is connected to the positive side of the circuit, but also to work quite well on "straight polarity", or when it is connected to the negative side of the circuit—a versatility of operation which is unusual.

5 I claim as my invention:—

1. A weld-rod having a coating containing ilmenite, mica, and a binder silicate, with each of the first two forming from 10% to 40% of the total of the three.

2. A weld-rod having a coating containing ilmenite, mica, and a binder silicate, with each of the first two forming substantially one-fourth of the total of the three.

10 15 20 25 PAUL R. JUDY.